

## UNITED STATES PATENT OFFICE

1,924,245

## PROCESS FOR IMPROVING NICKEL-MOLYBDENUM ALLOYS

Werner Köster, Dortmund, Germany, assignor to  
the firm Vereinigte Stahlwerke Aktiengesellschaft,  
Düsseldorf, Germany

No Drawing. Application March 9, 1931, Serial  
No. 521,394, and in Germany July 4, 1930

2 Claims. (Cl. 148—11.5)

This invention relates to nickel-molybdenum alloys.

It has been ascertained by exhaustive experiments that nickel-molybdenum alloys can be hardened by a special heat treatment. If rolled or cast alloys containing 8 to 30% of molybdenum be heated to a temperature above about 900° C. and thereupon cooled with sufficient rapidity in air or by immersion in water or oil and finally heated to temperatures between 400° to 800° C., then the mechanical properties of the alloys will be very substantially increased in relation to those prior to said heat treatment.

If for example, an alloy containing 75% of nickel and 25% of molybdenum be heated to 1100° C., quenched in water and annealed for one hour at 600° C. the hardness increases from 260 Brinell in the untreated state to 368 Brinell.

It is to be understood that certain quantities of other metals such as Cu, Al, Fe, Co, Cr, Mn or non-metallic substances, may be combined with the binary alloys described, such as will not injuriously affect the nature of such alloys and which may to some extent modify their properties and render them more suitable for

special requirements, without however affecting their ability to precipitation hardening, depending upon the fact that the principal part of the alloys consists of nickel and molybdenum. Thus when in the ensuing claims I use the phrase "the balance substantially nickel", I intend that the content of nickel and molybdenum shall be not less than about 85% of the whole.

I claim:

1. A process for obtaining alloys of high hardness consisting in forming an alloy of 8 to 30% of molybdenum and the balance chiefly nickel and heating said alloy to a temperature lying between 900° C. and the melting point of the alloy, then rapidly cooling said alloy and subsequently annealing it at temperatures between 400 and 800° C. 65

2. An alloy containing 8 to 30% of molybdenum and the balance principally nickel, having high hardness produced by heating the alloy 75 to a temperature lying between 900° C. and the melting point of the alloy, then rapidly cooling said alloy and subsequently annealing it at a temperature between 400 and 800° C. 70

WERNER KÖSTER. 80

30

85

35

90

40

95

45

100

50

105

55

110